# EUROPEAN PATENT SPECIFICATION

(11) **EP 0 785 296 B1**
(45) Date of publication and mention of the grant of the patent: **15.03.2000**
(21) Application number: 96309396.8
(22) Date of filing: 23.12.1996
(51) Int. Cl.: C25D 3/12

(54) **Electroplating of nickel on nickel ferrite devices**
Elektroplattieren von Nickel auf Nickel-Ferrit Vorrichtungen
Dépôt électrolytique de nickel sur des dispositifs en nickel ferrite

(30) Priority: 29.12.1995 US 581079; 18.12.1996 US 769189
(43) Date of publication of application: 23.07.1997
(73) Proprietor: AT&T Corp., New York, NY 10013-2412 (US)
(72) Inventor: Law, Henry Hon, Berkeley Heights, New Jersey 07922 (US); Wu, Te-Sung, New Providence, New Jersey 07974 (US); Schneemeyer, Lynn Frances, Westfield, NJ 07090 (US)
(74) Representative: Johnston, Kenneth Graham

(56) References cited:
- US-A- 3 620 936
- US-A- 3 960 674
- US-A- 4 375 390
- CHEMICAL ABSTRACTS, vol. 120, no. 12, 21 March 1994 Columbus, Ohio, US; abstract no. 147161h, ZUO ZHENZHONG: "Non-boric acid bright nickel electroplating" XP002029499 & CAILIAO BAOHU, vol. 26, no. 1, 1993, page 4-9

## Description

This invention relates to electroplating and, in particular, to electroplating a nickel layer on a nickel ferrite device.

### Background of the Invention

In the manufacture of circuits containing magnetic components, it is sometimes necessary to electroplate a nickel layer on conductors disposed on a nickel ferrite substrate. For example, in the fabrication of integrated power modules it is desirable to electroplate nickel onto copper conductors disposed on nickel zinc ferrite substrates. The nickel-plated conductors provide a surface that is wire-bondable with aluminum wire so that additional components can be directly connected to circuit components on the ferrite substrate.

While the technology of nickel plating is generally well established, excessive lateral growth is encountered in the conventional plating of nickel on nickel ferrite substrates. For example, in coating about 2µm of nickel on ferrite-supported copper conductors, over 100µm of lateral nickel growth was observed. Such lateral growth is highly deleterious in the fabrication of circuit devices because adjacent conductors can be shorted. Moreover such lateral growth precludes the fabrication of high density circuits having tightly-spaced conductor lines. Accordingly there is a need for a new method of electroplating nickel on nickel ferrite substrates.

U.S. 3,960,674 discloses a process of electroplating nickel on to conductive metal patterns formed on a non-conductive ferrite substrate.

According to the present invention there is provided a method as defined in claim 1.

This invention is predicated on the discovery by the present applicants that boric acid in conventional nickel plating baths is responsible for excessive lateral growth in the electroplating of nickel on nickel ferrite substrates. While nickel baths without boric acid do not yield acceptable electrodeposits, the boric acid interacts with the ferrite substrate to cause excessive lateral growth. Applicants further discovered that by eliminating the boric acid and adding another acidic plating buffer such as citric acid, one can obtain isotropic nickel plating and produce a wire-bondable surface.

### Brief Description of the Drawings

The advantages, nature and various additional features of the invention will appear more fully upon consideration of the illustrative embodiment described in connection with the accompanying drawings. In the drawings:
FIG. 1 is a schematic cross section of a plated nickel ferrite substrate subject to excessive lateral growth; and
FIG. 2 is a schematic cross section of a nickel ferrite substrate plated in accordance with a preferred embodiment of the invention.

It is to be understood that these drawings are for purposes of illustrating the concepts of the invention and are not to scale.

### Detailed Description

Referring to the drawings, FIG. 1 is a schematic cross section of a nickel ferrite substrate 10, such as nickel zinc ferrite, bearing a conductor 11, such as copper. A coating of nickel 12 has been coated on the conductor using a conventional nickel plating bath. As illustrated, the plated nickel on either side of the conductor 11 extends substantially farther than the thickness of the nickel on top of the conductor. This lateral extension illustrates excessive lateral growth, and one can readily see that such growth limits the close spacing of conductors.

As specific examples, applicants observed plating patterns similar to FIG. 1 using a conventional Barrett nickel sulfamate bath. Two µm of nickel were plated on two parallel copper conductor lines spaced about 360µm apart on a nickel zinc ferrite substrate. Plating was at a current density of 20 mA/cm² for 5 minutes. About 150µm of nickel deposited on each side of the conductor, giving a vertical-to-lateral ratio of about 0.013. Reducing the plating time by increasing the plating current density did not eliminate the excessive lateral growth. Nor did plating with a different commercial bath, Sulfamtronics.

To investigate whether the boric acid contributed to the lateral growth, samples were plated with nickel using nickel sulfamate baths containing various amounts of boric acid ranging from 30 g/L to below 2 g/L. It was found that at a boric acid concentration of 2 g/L or lower, lateral growth was not observed. However, the resulting nickel coating was not wire-bondable to aluminum.

Since common nickel plating baths use boric acid as a buffering agent to prevent the formation of Ni (OH)₂ at the cathode interface and to prevent the formation of hydrogen, applicants formulated new buffered plating baths substantially free of boric acid (less than 2 g/L).

FIG. 2 is a schematic cross section of a nickel ferrite substrate 20 bearing a metal conductor 21 electroplated with nickel 22 from a buffered nickel plating bath free of boric acid. As illustrated, the lateral growth of nickel is substantially the same as the vertical growth, so the plating is isotropic.

The nickel ferrite substrate 20 can comprise any nickel-containing ferrite, but is preferably a ferrite of the form Ni₁₋ₓZnₓFe₂O₄, NiFe₂₋ₓAlₓO₄ and Ni₁₋ₓCdₓFeₓO₄ where x can vary from zero to nearly 1. The metal conductor 21 can be any metal which can be adhered to the nickel-ferrite substrate as by co-firing (silver-palladium) or by electroplating to a co-fired metal (e.g., copper electroplated to silver-palladium alloy). The nickel plating bath comprises a solution of nickel salt in an acidic buffer having a pH of about 3 or less which contains less than 2 g/L of boric acid. It is possible to use any acidic buffer that provides a pH in this range. Preferred nickel salts include nickel sulfate, nickel sulfamate, nickel chloride and nickel fluoroborate. Preferred acidic buffers include citric acid, acetic acid, phosphoric acid, succinic acid, glycolic acid, and tartaric acid.

### Example 1

A nickel plating bath was made of the following composition:

| Compound | Amount (g/L) |
|---|---|
| Ni(SO₃NH₂)₂·4H₂O | 383 |
| NiCl₂·6H₂O | 11 |
| Citric Acid | 10 |

Nickel ferrite samples with copper conductors were plated at (22mA/cm²) with a pH of about 1.9 and a temperature in the range 35-45°C. No lateral growth was observed. The sample was plated to a thickness of 20µm. Lateral growth was measured to be about 20µm, which means that plating was isotropic. The appearance was acceptable, and the coating was wire-bondable to aluminum wire.

### Examples 2-8

Nickel plating baths having the same type and concentration of nickel salts as Example 1, but with the buffers indicated below, were prepared. Nickel ferrite samples with copper conductors (pre-plated for IS minutes at 27mA/cm²) were also prepared and plated with nickel in the baths at 35°C. Table I below indicates the concentration of buffer, the plating current, the pH of the bath, whether the nickel exhibited excessive lateral growth (i.e., anisotropic growth), and whether the nickel coating was wire-bondable to aluminum.

**TABLE I**

| Buffer | Buffer Concen. | mA/cm² | Plating Current | Bath pH | Excessive Lateral Growth | Wire-Bondable |
|---|---|---|---|---|---|---|
| Boric acid | 10 g/L | 16 | (15 A/ft²) | 3.9 | Yes | Yes |
| Succinic acid | 10 g/L | 16 | (15 A/ft²) | 2.22 | No | Yes |
| Glycolic acid | 10 g/L | 19 | (18 A/ft²) | 1.68 | No | Yes |
| Tartaric acid | 10 g/L | 19 | (18 A/ft²) | 1.71 | No | Yes |
| Formic acid | 10 g/L | 13 | (12 A/ft²) | 4.88 | Yes | not attempted |
| Acetic acid | 10 g/L | 16 | (15 A/ft²) | 1.72 | No | Yes |
| Phosphoric acid | 5 g/L | 8 | (7 A/ft²) | 2.36 | No | Yes |

## Claims

1. A method of electroplating nickel on a nickel ferrite device comprising the steps of:
providing a substrate of nickel-containing ferrite;
adhering a metal conductor to said substrate;
disposing said substrate and said conductor in a nickel plating bath comprising nickel salt and an acidic buffer substantially free of boric acid for buffering said bath to a pH of about 3 or less; and
applying an electric current through said conductor to isotropically electroplate a desired thickness of nickel on said conductor.

2. The method of claim 1 wherein said nickel-containing ferrite comprises a ferrite selected from the group consisting of Ni₁₋ₓZnₓFe₂O₄, NiFe₂₋ₓAlₓO₄ and Ni₁₋ₓCdₓFe₂O₄, where 0 < x < 1.

3. The method of claim 1 wherein said metal comprises copper.

4. The method of claim 1 wherein said metal comprises silver palladium alloy.

5. The method of claim 1 wherein said nickel salt comprises a nickel salt selected from the group consisting of nickel sulfate, nickel sulfamate, nickel chloride and nickel fluoroborate.

6. The method of claim 1 wherein said acidic buffer comprises a buffer selected from the group consisting of citric acid, acetic acid, phosphoric acid, succinic acid, glycolic acid, and tartaric acid.

## Patentansprüche

1. Verfahren zum Elektroplattieren von Nickel auf eine Nickel-Ferrit-Vorrichtung mit folgenden Schritten:
ein Substrat mit Ferrit, welches Nickel umfaßt, wird bereitgestellt;
ein metallischer Leiter wird an das Substrat anhaften lassen;
das Substrat und der Leiter werden in ein Nickel-Plattierungsbad eingetaucht, welches Nickel-Salz und eine Puffersäure, die im wesentlichen frei von Borsäure ist, umfaßt, um das Bad auf einen pH-Wert von etwa 3 oder weniger zu puffern;
ein elektrischer Strom wird durch den Leiter fließen lassen, um eine gewünschte Dicke des Nickels an dem Leiter isotropisch zu elektroplattieren.

2. Verfahren nach Anspruch 1, dadurch gekennzeichnet, daß das Ferrit, welches Nickel aufweist, ein Ferrit umfaßt, das aus einer Gruppe gewählt wird, die aus Ni₁₋ₓZnₓFe₂O₄, NiFe₂₋ₓAlₓO₄ und Ni₁₋ₓCdₓFe₂O₄ besteht, wobei 0<X<1.

3. Verfahren nach Anspruch 1, dadurch gekennzeichnet, daß das Metall Kupfer umfaßt.

4. Verfahren nach Anspruch 1, dadurch gekennzeichnet, daß das Metall eine Silber-Palladium-Legierung umfaßt.

5. Verfahren nach Anspruch 1, dadurch gekennzeichnet, daß das Nickel-Salz ein Nickel-Salz umfaßt, das aus der Gruppe gewählt wird, die Nickelsulfat, Nickelsulfamat, Nickelchlorid und Nickelfluroprochat umfaßt.

6. Verfahren nach Anspruch 1, dadurch gekennzeichnet, daß die Puffersäure einen Puffer umfaßt, der aus der Gruppe gewählt wird, die Zitronensäure, Essigsäure, Phosphorsäure, Bernsteinsäure, Glycolsäure und Weinsäure umfaßt.

## Revendications

1. Procédé d'électrodéposition de nickel sur un dispositif en nickel ferrite comportant les étapes qui consistent à :
prendre un substrat de ferrite contenant du nickel;
faire adhérer un conducteur métallique au substrat ;
disposer le substrat et le conducteur dans un bain de dépôt de nickel comportant du sel de nickel et un tampon acide sensiblement sans acide borique pour former le bain sous la forme d'un tampon à un pH d'environ 3 ou moins ; et
appliquer un courant électrique dans le conducteur pour électrodéposer de manière isotrope une épaisseur souhaitée de nickel sur le conducteur.

2. Procédé suivant la revendication 1, dans lequel le ferrite contenant du nickel comprend un ferrite sélectionné parmi le groupe constitué du Ni₁₋ₓZnₓFe₂O₄, NiFe₂₋ₓAlₓO₄ et Ni₁₋ₓCdₓFeₓO₄ où 0 < x < 1.

3. Procédé suivant la revendication 1, dans lequel le métal comprend du cuivre.

4. Procédé suivant la revendication 1, dans lequel le métal comprend un alliage d'argent et de palladium.

5. Procédé suivant la revendication 1, dans lequel le sel de nickel comprend un sel de nickel sélectionné parmi le groupe constitué de sulfate de nickel, de sulfamate de nickel, de chlorure de nickel et de fluoborate de nickel.

6. Procédé suivant la revendication 1, dans lequel le tampon acide comprend un tampon sélectionné parmi le groupe constitué de l'acide citrique, l'acide acétique, l'acide phosphorique, l'acide succinique, l'acide glycolique et l'acide tartrique.
